

No. 629,427.

Patented July 25, 1899.

G. D. COLEMAN.  
ANTIFOULING COATING FOR WOOD.

(Application filed Nov. 9, 1898.)

(No Model.)



FIG. 1.



FIG. 2.

WITNESSES

L. Kitching  
& E. Shylto.

INVENTOR

George D. Coleman,  
By his attorneys,  
Phillip & Anderson.

# UNITED STATES PATENT OFFICE.

GEORGE D. COLEMAN, OF BRIDGEWATER, MASSACHUSETTS.

## ANTIFOULING COATING FOR WOOD.

SPECIFICATION forming part of Letters Patent No. 629,427, dated July 25, 1899.

Application filed November 9, 1898. Serial No. 695,948. (No specimens.)

*To all whom it may concern:*

Be it known that I, GEORGE D. COLEMAN, a citizen of the United States, residing at Bridgewater, in the county of Plymouth and State of Massachusetts, have invented certain new and useful Improvements in Antifouling Coatings for Wood; and I do hereby declare the following to be a full, clear, and exact description of the invention, such as will enable others skilled in the art to which it appertains to make and use the same.

The object of my invention is to produce an efficient antifouling coating for wood, and especially an antifouling coating for the wooden bottoms of sea-going vessels and for the submerged portions of docks and the like, which are in contact with the sea-water and which in the absence of some antifouling coating are rapidly covered with marine growths, especially in the tropical seas, which in the case of vessels materially diminishes their speed.

In the drawings accompanying this specification, illustrating the preferred form of my invention, and in which like reference-letters refer to like parts throughout, Figure 1 is a face view, on a very much enlarged scale, of a portion of a piece of wood provided with indentations. Fig. 2 represents a cross-section, on the same scale, of a portion of a piece of wood with my antifouling coating applied thereto.

Heretofore it has been customary to coat the bottoms of ships with sheet-copper, which being exposed to the action of the sea-water is oxidized on its outer surface, and the oxids thus formed change to various other salts of copper, which being highly poisonous in their nature prevent the accumulation of marine growths thereon. My invention contemplates a substitute for such copper surface which shall be easily applied, efficiently held, and at the same time made very much more cheaply than the sheet-copper coating.

In carrying my invention into practice I apply to the surface of the wood comminuted copper, which is embedded therein. The portions of the particles of comminuted copper which remain exposed upon the surface of the wood become oxidized by contact with the sea-water, and the oxids thus formed gradually change into other salts of copper, which

efficiently prevent the accumulation of marine growths upon the surface of the wood.

While I have referred to comminuted copper as the material to be applied to and embedded in the surface of the wood, I do not desire to limit myself specifically to that metal, as it will be readily understood that any alloy of copper or other metal which upon exposure to the action of sea-water becomes rapidly coated with salts poisonous to marine growths is within the purview of my invention. So when I use the term "copper" I would have it understood that I may use that metal or its alloys or any other metal or alloy which decomposes in like manner.

The comminuted copper may be applied to the surface of the wood by being laid thereon and driven by suitable tools into the same. I prefer, however, to apply the comminuted copper to the surface of the wood after the same shall have been subjected to the action of tools which shall cut numerous indentations through the outer surface of the wood. Into these indentations I then drive the comminuted copper. As is well known, when dry wood is indented and afterward moistened a swelling of the fiber of the wood tends to obliterate the indentations by bringing the fiber to the surface again, so if the copper were merely driven into the smooth surface of the wood it might be that when the wood was moistened by immersion in water the particles of copper might be thrown off. In order to prevent this shedding of the particles of copper, I consider that it is preferable previously to cut indentations in the wood. By this means the continuity of the surface fiber of the wood is destroyed, and when the copper is embedded in the previously-formed indentations it will be securely held by the wood when the wood shall be moistened, because the swelling of the fiber by reason of the moisture will not act to shed or throw off the particles of copper, but the fiber will swell around them and hold them securely in the surface of the wood.

It is not necessary that the particles of copper should completely cover the entire surface of the wood, for the reason that as the copper decomposes under the action of the sea-water the salts thereby formed will spread around each particle of copper upon the contiguous

surfaces of the wood, covering the whole surface with a coating of poisonous salts, to which marine growths will not attach themselves.

Although it is quite practical and within the purview of my invention to apply the comminuted copper directly to the indented surface of the wood and to hammer the same therewith, I have found it convenient and preferable to apply the comminuted copper to the surface of the wood in a paste soluble in water. By this means I am enabled to apply to the surface of the wood a coating of comminuted copper in position to be driven into the surface of the wood by a hammer or any other suitable tool. After the hammering process is completed the soluble paste may be washed off, and thus affords a ready means of examining the surface and determining as the work progresses the closeness of the particles of copper to each other.

In case the comminuted copper is applied directly to the wood without the use of a paste or after the paste has been washed off and the surface of the wood is exposed it will be found to be provided with a coating of many small pieces of copper embedded in the wood. This coating is an efficient one for the prevention of accumulation of marine growths; but I prefer at this stage to coat the whole with a paint composed of the poisonous salts of copper, which paint efficiently fills the interstices between the small particles of copper and at the same time promotes the decomposition of these particles when subjected to the action of sea-water. This paint of the poisonous salts of copper may be any of the well-known antifouling paints or a paint entirely of such poisonous salts of copper or any material which will become poisonous on exposure to sea-water in the presence of copper and any desired volatile binder which will serve to tie the substance together until it shall become hard and dry. It may be applied with a brush or with a trowel, depending upon its consistency and the amount desired to be applied, and the surface may be smoothed in any suitable or desired manner. When wood coated in the above manner is subjected to the action of sea-water, the antifouling substance which fills the interstices between the embedded particles of comminuted copper will of course gradually be abraded and washed off by the action of the water; but the particles of copper being at the same time subjected to the action of the sea-water will be decomposed and serve to renew the antifouling substance lost from between the particles of comminuted copper.

In Fig. 1 of the drawings I have illustrated

a portion of the surface of the wood provided with indentations A to receive the particles of comminuted copper, and in Fig. 2 I have shown a cross-section of a portion of a piece of wood B through the coating, wherein C indicates the particles of comminuted copper and D indicates the surface coating of antifouling substance in the interstices between the particles of comminuted copper. This figure clearly shows, on a much-enlarged scale, the embedding of the particles of copper in the surface of the wood.

I am aware that it is old to apply a coating to the bottoms of ships which consists of a paint, such as red lead, having suspended therein particles of comminuted copper; but it will be observed that such coating is radically different from the coating which I apply, and, moreover, it is liable to be chipped or flaked off from the bottom of the vessel by accidental contact with flotsam, while my coating, being attached at every point to the surface of the wood, is not liable to scale or chip off, but in case of injury thereto the injury is confined to the precise spot struck, besides which the copper being embedded in the wood cannot be easily removed therefrom by such chance blows, and even if the surface were severely indented would still present antifouling material to the water, and thereby prevent the accumulation of marine growths. In other words, the comminuted copper applied according to my invention makes a very much more durable coating by reason of its being embedded in the surface of the wood and not merely attached thereto by force of cohesion and having the further advantage of renewing itself by decomposition of the metallic copper.

Having thus described my invention, I claim as broadly novel and desire to secure by Letters Patent of the United States—

1. An antifouling coating for wood which consists of comminuted copper or other suitable substance embedded in the surface of the wood, substantially as described.

2. An antifouling coating for wood which consists of comminuted copper or other suitable substance embedded in the surface of the wood and a surface coating of antifouling substance in the interstices between the embedded particles of comminuted substance, substantially as described.

In testimony whereof I affix my signature in presence of two witnesses.

GEORGE D. COLEMAN.

Witnesses:

T. HART ANDERSON,  
HORACE VAN EVEREN.